# EUROPEAN PATENT SPECIFICATION

(11) **EP 0 757 712 B1**
(45) Date of publication and mention of the grant of the patent: **22.03.2000**
(21) Application number: 95916764.4
(22) Date of filing: 25.04.1995
(51) Int. Cl.: C10M 169/04

(54) **LUBRICANT COMPOSITION**
SCHMIERMITTELZUSAMMENSETZUNG
COMPOSITION DE LUBRIFIANT

(30) Priority: 26.04.1994 GB 9408235
(43) Date of publication of application: 12.02.1997
(73) Proprietor: CASTROL LIMITED, Swindon, Wiltshire SN3 1RE (GB)
(72) Inventor: MARKSON, Andrew, Jonathan, Upper Basildon Reading RG8 8TA (GB); PRAGNELL, John, William, Anthony, Whitchurch Hill Pangbourne RG8 7PZ (GB); EDWARDS, Mark, Anthony, Binfield Berkshire RG42 4UT (GB)
(74) Representative: Lewis, Pauline Therese
(86) International application number: GB9500941
(87) International publication number: WO9529214

(56) References cited:
- WO-A-94/10270
- DE-A- 2 039 785
- FR-A- 2 215 462
- US-A- 3 694 382

## Description

This invention relates to a lubricant composition and is particularly concerned with a transmission lubricant suitable, for example, for helicopter transmission systems.

The development of new transmission systems, for example, for helicopters, has led to the requirement for dedicated lubricants for such purposes which can meet demanding load carrying and corrosion protection criteria. Specifications put forward by, for example, the U.K. Ministry of Defence and the United States Navy, pose requirements to be met by new dedicated helicopter transmission lubricants that cannot be fulfilled by existing aviation turbine engine lubricants. There is thus a need for the development of new and improved lubricant compositions for such purposes. The present invention seeks to fulfil this need.

DE-A-2039785 discloses a load carrying additive composition for a gas turbine engine. The load carrying additive composition comprises a synthetic ester base stock fluid having a viscosity of 5.6 to 6.0 cs. at 99 °C (210 °F) (see the examples).

US-A-3694382 discloses a lubricant for a gas turbine engine. The lubricant comprises a synthetic ester base stock having a viscosity ranging from 4.0 to 9.1 cs. at 99 °C (210 °F).

FR-A-2215462 discloses a lubricant having a mineral oil as its base stock.

WO-A-9410270 discloses a corrosion inhibiting lubricating composition comprising a synthetic base stock having a viscosity of at least 4.9 cSt at 100 °C.

In this document, reference is made to 'IRGALUBE®' and 'Herco A®', both of which may be registered trade marks.

Accordingly, the present invention provides a lubricant composition comprising:
a) a base component comprising one or more synthetic base stocks, which base component has a viscosity in the range of from 8.5 to 9.5 mm²/s (cSt) at 100°C;
b) at least one antioxidant selected from aromatic amines and hindered phenolics;
c) at least one neutral organic phosphate of the formula (R¹O)₃PO where R¹ is a tolyl, phenyl, xylyl, alkyl or cycloalkyl group, the alkyl or cycloalkyl group having up to 10 carbon atoms; the neutral organic phosphate being present in an amount from 1.5 to 2.5% by weight of the composition;
d) at least one saturated and/or unsaturated dicarboxylic acid of the general formula wherein $\text{x+y+z}$ is an integer in the range from 2 to 22 inclusive and where at least one of the groups R₁ to R₅ is a carboxylic acid group and the remaining groups R₁ to R₅ are selected from alkyl, hydroxy, nitro, amino, carboxyl, hydrogen or alkyl derivatives thereof, where alkyl is a short chain of up to 5 carbon atoms; and/or a dicarboxylic acid of one of the three formulae wherein R'₁ is -COOH, alkyl, hydroxy, nitro, amino, hydrogen or alkyl derivatives thereof; R'₂ is -COOH; and n is an integer from 1 to 4 inclusive when R'₁ is -COOH or an integer from 2 to 4 inclusive when R'₁ is not -COOH.
e) at least one straight and/or branched chain saturated or unsaturated monocarboxylic acid which is optionally sulphurised in an amount which may be up to 35% by weight; and/or an ester of such an acid; and
f) at least one triazole of the formula: where R''₁ is -COOH or alkyl derivatives thereof, or short chain alkyl of up to 5 carbon atoms; n is zero or an integer between 1 and 3 inclusive; and R''₂ is hydrogen, morphilino, alkyl, amido, amino, hydroxy or alkyl or aryl substituted derivatives thereof; or a triazole selected from 1,2,4 triazole, 1,2,3 triazole, 5-anilo-1,2,3, 4-thiatriazole, 3-amino-1,2,4 triazole, 1-H-benzotriazole- 1-yl-methylisocyanide, methylene-bis-benzotriazole and naphthotriazole; and
g) at least one phosphorus containing extreme pressure additive.

In component (d) above the bicyclic structural formula is intended to indicate that the group(s) R₂ may be attached to either or both aromatic rings.

At least one base stock of the base component, is preferably a synthetic ester base stock, especially a polyol ester base stock. The synthetic polyolester which preferably forms a base stock of the lubricating composition of the present invention may be made from C₅ to C₁₂ monocarboxylic acids esterified with polyols or polyol ethers such as neopentylglycol, dimethylolpropane, trimethylolpropane, pentaerythritol or dipentaerythritol. These are conventional synthetic ester base stocks. Preferred esters are those which are described in U.S. Patent 4826633.

The viscosity may be adjusted to lie within the required range by inclusion of one or more viscosity index improvers.

For adequate performance as a transmission lubricant, the base component must have a viscosity in the range of 8.5 to 9.5 cSt, preferably 8.75 to 9.25 mm²/s (cSt), at 100°C. The base component may comprise a single polyol ester but is more usually a mixture of polyol esters, for example, a mixture of a polyol ester having a viscosity of about 4.0 cSt at 100°C with a polyol ester having a viscosity of about 12.0 mm²/s (cSt) at 100°C. Preferred synthetic polyol esters are reaction products of pentaerythritol and/or trimethylolpropane and an acid mixture comprising C₅ to C₁₀ straight and branched chain acids.

The antioxidant component b) may be a hindered phenolic antioxidant such as butylated hydroxytoluene, suitably present in an amount of 0.01 to 5%, preferably 0.4 to 0.8%, by weight of the lubricant composition. Alternatively, or in addition, component b) may comprise an aromatic amine antioxidant such as mono-octylphenylalphanapthylamine or p,p-dioctyldiphenylamine, used singly or in admixture. The amine anti-oxidant component is suitably present in a range of from 0.01 to 5% by weight of the lubricant composition, more preferably 0.5 to 1.5%.

The neutral organic phosphate which forms component c) of the formulation is present in an amount of 1.5 to 2.5% by weight of the composition. The neutral organic phosphate is also a conventional ingredient of lubricating compositions and any such neutral organic phosphate falling within the formula as previously defined may be employed. Tri-cresyl phosphate is a preferred phosphate for use in the present invention.

Components d), e) and f) are intended to provide a corrosion inhibiting three component system. The combination has been found to enable the provision of lubricant compositions capable of passing United States Navy corrosion inhibition requirements (Ball Corrosion Test - ARP 4249) in which a result of 50% non corroded specimen is deemed a satisfactory corrosion protection requirement.

The dicarboxylic acid forming the first component of the anti-corrosion combination may be any dicarboxylic acid falling within the definition given hereinbefore. The dicarboxylic acid may be present in a proportion of up to 0.15% by weight of the composition. It should be noted however, that it is desirable that sebacic acid or an equivalent thereof should always be present in the composition even if another dicarboxylic acid falling within the above definition is present because sebacic acid or an equivalent of it may be necessary to meet parts of the specification other than the ball corrosion test, for example, for satisfactory lead corrosion resistance.

Examples of dibasic acids, other than sebacic acids, which may be used in the present invention, are adipic acid, azelaic acid, dodecanedioic acid, 3-methyladipic acid, 3-nitrophthalic acid, 1,10-decanedicarboxylic acid, and fumaric acid.

The second component of the anti-corrosion combination is a straight or branch-chained, saturated or unsaturated monocarboxylic acid or ester thereof which may optionally be sulphurised in an amount up to 35% by weight. Preferably the acid is a C₄ to C₂₂ straight chain unsaturated monocarboxylic acid. The preferred concentration of this additive is from 0.001% to 0.35% by weight of the total lubricant composition. The preferred monocarboxylic acid is sulphurised oleic acid. However, other suitable materials are oleic acid itself; valeric acid and erucic acid.

The third component of the anti-corrosion combination is a triazole as previously defined. The triazole should be used at a concentration from 0.005% to 0.25% by weight of the total composition. The preferred triazole is benzotriazole.

Component g) of the composition comprises at least one phosphorus containing extreme pressure additive. Examples of such additives are amine phosphate extreme pressure additives such as that known under the trade name *IRGALUBE® 349* and/or triphenyl phosphorothionate extreme pressure/anti-wear additives such as that known under the trade name *IRGALUBE® TPPT*. Such amine phosphates are suitably present in an amount of from 0.01 to 2%, preferably 0.2 to 0.6% by weight of the lubricant composition while such phosphorothionates are suitably present in an amount of from 0.01 to 3%, preferably 0.5 to 1.5% by weight of the lubricant composition. Preferably, a mixture of an amine phosphate and phosphorothionate is employed.

For the provision of a helicopter transmission lubricant the amounts of the additive are selected so as to comply with the United States Navy requirement for the Ryder gear test, conducted at 100°C, (average of 6 runs) of 200 (relative rating, % Herco® A as reference fluid).

The following example is intended to illustrate a preferred lubricant composition in accordance with the invention.

| | % by weight |
|---|---|
| mono-octylphenylalphanaphthylamine | 0.5% |
| butylated hydroxy toluene | 0.5% |
| benzotriazole | 0.1% |
| sulphurised oleic acid | 0.05% |
| sebacic acid | 0.01% |
| tri-cresyl phosphate | 2.0% |
| amine phosphate | 0.4% |
| triphenyl phosphorothionate | 1.0% |
| silicone antifoam agent | 2ppm |
| base synthetic ester fluid mixture to give a viscosity for the composition of 8.75 to 9.25 mm²/s (cSt) | 95.44% |

The resulting composition was found to give a value of 204.7 in the Ryder gear test, 100°C (as relative rating, % Herco® A) and pass rating in the Ball Corrosion Test (in accordance with ARP method 4249).

## Claims

1. A lubricant composition comprising:
a) a base component comprising one or more synthetic base stocks, which base component has a viscosity in the range of from 8.5 to 9.5 mm²/s (cSt) at 100°C;
b) at least one antioxidant selected from aromatic amines and hindered phenolics;
c) at least one neutral organic phosphate of the formula (R¹O)₃PO where R¹ is a tolyl, phenyl, xylyl, alkyl or cycloalkyl group, the alkyl or cycloalkyl group having up to 10 carbon atoms; the neutral organic phosphate being present in an amount from 1.5 to 2.5% by weight of the composition;
d) at least one saturated and/or unsaturated dicarboxylic acid of the general formula wherein $\text{x+y+z}$ is an integer in the range from 2 to 22 inclusive and where at least one of the groups R₁ to R₅ is a carboxylic acid group and the remaining groups R₁ to R₅ are selected from alkyl, hydroxy, nitro, amino, carboxyl, hydrogen or alkyl derivatives thereof, where alkyl is a short chain of up to 5 carbon atoms; and/or a dicarboxylic acid of one of the three formulae wherein R'₁ is -COOH, alkyl, hydroxy, nitro, amino, hydrogen or alkyl derivatives thereof; R'₂ is -COOH; and n is an integer from 1 to 4 inclusive when R'₁ is -COOH or an integer from 2 to 4 inclusive when R₁ is not -COOH.
e) at least one straight and/or branched chain saturated or unsaturated monocarboxylic acid which is optionally sulphurised in an amount which may be up to 35% by weight; and/or an ester of such an acid; and
f) at least one triazole of the formula: where R''₁ is -COOH or alkyl derivatives thereof, or short chain alkyl of up to 5 carbon atoms; n is zero or an integer between 1 and 3 inclusive; and R''₂ is hydrogen, morphilino, alkyl, amido, amino, hydroxy or alkyl or aryl substituted derivatives thereof; or a triazole selected from 1,2,4 triazole, 1,2,3 triazole, 5-anilo-1,2,3, 4-thiatriazole, 3-amino-1,2,4 triazole, 1-H-benzotriazole-1-yl-methylisocyanide, methylene-bis-benzotriazole and naphthotriazole; and
g) at least one phosphorus containing extreme pressure additive.
wherein components (b) to (g) are present in amounts selected so as to comply with the United States Navy requirement for Ryder gear test, conducted at 100°C, of 200 (relative rating, % Herco® A as reference fluid)

2. A lubricant composition according to claim 1 wherein at least one base stock of the base component is a polyol ester.

3. A lubricant composition according to claim 2 wherein the polyol ester base stock comprises one or more C₅ to C₁₂ monocarboxylic acids esterified with one or more polyols or polyol ethers.

4. A lubricant composition according to anyone of claims 1 to 3 wherein the base component has a viscosity in the range of from 8,75 to 9.25 mm²/s (cSt) at 100°C.

5. A lubricant composition according to any one of the preceding claims wherein the antioxidant comprises a hindered phenolic antioxidant present in an amount of 0.4 to 0.8% by weight of the composition.

6. A lubricant composition according to anyone of the preceding claims wherein the antioxidant comprises an aromatic amine antioxidant present in an amount of 0.5 to 1.5% by weight of the composition.

7. A lubricant composition according to any one of the preceding claims wherein the saturated and/or unsaturated dicarboxylic acid component (d) is present in an amount of up to 0.15% by weight of the composition.

8. A lubricant composition according to any one of the preceding claims wherein the saturated and/or unsaturated dicarboxylic acid component (d) comprises sebacic acid.

9. A lubricant composition according to any one of the preceding claims wherein the monocarboxylic and component (e) is present in an amount of from 0.001 to 0.35% by weight of the composition.

10. A lubricant composition according to any one of the preceding claims wherein the monocarboxylic acid component (e) comprises sulphurised oleic acid.

11. A lubricant composition according to any one of the preceding claims wherein the triazole component (f) is present in an amount of from 0.005 to 0.25% by weight of the composition.

12. A lubricant composition according to any one of the preceding claims wherein the triazole component (f) comprises benzotriazole.

13. A lubricant composition according to any one of the preceding claims wherein the extreme pressure additive component (g) comprises an amine phosphate extreme pressure additive present in an amount of from 0.2 to 0.6% by weight of the composition.

14. A lubricant composition according to any one of the preceding claims wherein the extreme pressure additive component (g) comprises a phosphorothionate extreme pressure additive present in an amount of from 0.5 to 1.5% by weight of the composition.

15. A helicoptor transmission lubricant comprising components (a) to (g) as defined in any one of the preceding claims.

## Patentansprüche

1. Schmiermittelzusammensetzung, enthaltend
a) eine Basiskomponente, in der ein oder mehrere synthetische Grundmaterialien vorliegen und die eine Viskosität im Bereich von 8,5 bis 9,5 mm²/s (cSt) bei 100°C aufweist,
b) mindestens ein Antioxidationsmittel, das aus aromatischen Aminen und gehinderten Phenolen ausgewählt ist,
c) mindestens ein neutrales organisches Phosphat der Formel (R¹O)₃PO, in der R¹ einen Tolyl-, Phenyl-, Xylyl-, Alkyl- oder Cycloalkylrest bedeutet, wobei der Alkyl- oder Cycloalkylrest bis zu 10 Kohlenstoffatome enthält und wobei das neutrale organische Phosphat in einer Menge von 1,5 bis 2,5 Gew% der Zusammensetzung vorliegt,
d) mindestens eine gesättigte und/oder ungesättigte Dicarbonsäure der allgemeinen Formel worin $\text{x+y+z}$ eine ganze Zahl im Bereich von 2 bis 22 einschließlich sowie mindestens einer der Reste R₁ bis R₅ einen Carbonsäurerest bedeuten und die üblichen Reste R₁ bis R₅ aus Alkyl, Hydroxy, Nitro, Amino, Carboxyl, Wasserstoff oder Alkylderivaten hiervon ausgewählt sind, wobei Alkyl eine kurze Kette von bis zu 5 Kohlenstoffatomen darstellt, und/oder eine Dicarbonsäure mit einer der drei Formeln worin R'₁ die Gruppe -COOH, Alkyl, Hydroxy, Nitro, Amino, Wasserstoff oder ein Alkylderivat hiervon, R'₂ die Gruppe -COOH und n eine ganze Zahl von 1 bis 4 einschließlich, wenn R'₁ die Gruppe -COOH darstellt, oder eine ganze Zahl von 2 bis 4 einschließlich, wenn R'₁ nicht die Gruppe -COOH darstellt, bedeuten,
e) mindestens eine geradkettige und/oder verzweigtkettige gesättigte oder ungesättigte Monocarbonsäure, die gegebenenfalls in einer Menge, die bis zu 35 Gew% betragen kann, sulfuriert ist, und/oder einen Ester einer solchen Säure,
f) mindestens ein Triazol der Formel worin R''₁ die Gruppe -COOH oder ein Alkylderivat hiervon oder einen kurzkettigen Alkylrest von bis zu 5 Kohlenstoffatomen, n die Zahl 0 oder eine ganze Zahl zwischen 1 und 3 einschließlich und R''₂ Wasserstoff, Morpholino, Alkyl, Amido, Amino, Hydroxy oder Alkyl oder ein arylsubstituiertes Derivat hiervon oder ein Triazol, das aus 1,2,4-Triazol, 1,2,3-Triazol, 5-Anilino-1,2,3,4-thiatriazol, 3-Amino-1,2,4-triazol, 1-H-Benzotriazol-1-yl-methylisocyanid, Methylen-bis-benzotriazol und Naphthotriazol ausgewählt ist, und
g) mindestens ein phosphorhaltiges Extremdruckadditiv,
wobei die Komponenten b) bis g) in Mengen vorliegen, die derart gewählt sind, daß sie den Anforderungen der US-Marine für den Ryder-Getriebetest (Ryder gear test), durchgeführt bei 100°C, von 200 (relative Bewertung, % Herco® A als Bezugsfluid) entsprechen.

2. Schmiermittelzusammensetzung nach Anspruch 1, worin mindestens ein Grundmaterial der Basiskomponente ein Polyolester ist.

3. Schmiermittelzusammensetzung nach Anspruch 2, worin das Polyolester-Grundmaterial eine oder mehrere C₅- bis C₁₂-Monocarbonsäuren, verestert mit einem oder mehreren Polyolen oder Polyolethern, enthält.

4. Schmiermittelzusammensetzung nach einem der Ansprüche 1 bis 3, worin die Grundkomponente eine Viskosität im Bereich von 8,75 bis 9,25 mm²/s (cSt) bei 100°C aufweist.

5. Schmiermittelzusammensetzung nach einem der vorstehenden Ansprüche, worin das Antioxidationsmittel ein gehindertes phenolisches Antioxidationsmittel enthält, das in einer Menge von 0,4 bis 0,8 Gew% der Zusammensetzung vorliegt.

6. Schmiermittelzusammensetzung nach einem der vorstehenden Ansprüche, worin das Antioxidationsmittel ein Antioxidationsmittel in Form eines aromatischen Amins enthält, das in einer Menge von 0,5 bis 1,5 Gew% der Zusammensetzung vorliegt.

7. Schmiermittelzusammensetzung nach einem der vorstehenden Ansprüche, worin die gesättigte und/oder ungesättigte Dicarbonsäurekomponente (d) in einer Menge von bis zu 0,15 Gew% der Zusammensetzung vorliegt.

8. Schmiermittelzusammensetzung nach einem der vorstehenden Ansprüche, worin die gesättigte und/oder ungesättigte Dicarbonsäurekomponente (d) Sebacinsäure enthält.

9. Schmiermittelzusammensetzung nach einem der vorstehenden Ansprüche, worin die Monocarbonsäurekomponente (e) in einer Menge von 0,001 bis 0,35 Gew% der Zusammensetzung vorliegt.

10. Schmiermittelzusammensetzung nach einem der vorstehenden Ansprüche, worin die Monocarbonsäurekomponente (e) sulfurierte Ölsäure enthält.

11. Schmiermittelzusammensetzung nach einem der vorstehenden Ansprüche, worin die Triazolkomponente (f) in einer Menge von 0,005 bis 0,25 Gew% der Zusammensetzung vorliegt.

12. Schmiermittelzusammensetzung nach einem der vorstehenden Ansprüche, worin die Triazolkomponente (f) Benzotriazol enthält.

13. Schmiermittelzusammensetzung nach einem der vorstehenden Ansprüche, worin die Extremdruckadditiv-Komponente (g) ein Aminphosphat-Extremdruckadditiv enthält, das in einer Menge von 0,2 bis 0,6 Gew% der Zusammensetzung vorliegt.

14. Schmiermiittelzusammensetzung nach einem der vorstehenden Ansprüche, worin die Extremdruckadditiv-Komponente (g) ein Thiophosphatextremdruckadditiv enthält, das in einer Menge von 0,5 bis 1,5 Gew% der Zusammensetzung vorliegt.

15. Hubschraubergetriebeschmiermittel, enthaltend die Komponenten (a) bis (g), wie sie in einem der vorstehenden Ansprüche definiert sind.

## Revendications

1. Composition de lubrifiant comprenant :
a) un composant de base comprenant un ou plusieurs matériaux de base synthétiques, lequel composant de base présente une viscosité située dans l'intervalle allant de 8,5 à 9,5 mm²/s (cSt) à 100°C ;
b) au moins un antioxydant choisi parmi les amines aromatiques et les composés phénoliques stériquement encombrés ;
c) au moins un phosphate organique neutre de formule (R¹O)₃PO dans laquelle R¹ représente un groupe tolyle, phényle, xylyle, alkyle ou cycloalkyle, le groupe alkyle ou cycloalkyle comportant jusqu'à 10 atomes de carbone ; le phosphate organique neutre étant présent en une quantité de 1,5 à 2,5% en poids de la composition,
d) au moins un acide dicarboxylique saturé et/ou insaturé de formule générale dans laquelle $\text{x+y+z}$ représente un nombre entier dans l'intervalle allant de 2 à 22, bornes incluses, et dans laquelle au moins l'un des groupes R₁ à R₅ est un groupe acide carboxylique et les groupes R₁ à R₅ restants sont choisis parmi alkyle, hydroxy, nitro, amino, carboxyle, hydrogène, ou des dérivés alkylés de ceux-ci, le groupe alkyle étant une chaîne courte comportant jusqu'à 5 atomes de carbone ; et/ou un acide dicarboxylique répondant à l'une des trois formules dans lesquelles R'₁ représente -COOH, alkyle, hydroxy, nitro, amino, hydrogène, ou des dérivés alkylés de ceux-ci ; R'₂ représente -COOH ; et n représente un nombre entier de 1 à 4, bornes incluses, lorsque R'₁ représente -COOH, ou un nombre entier de 2 à 4, bornes incluses, lorsque R'₁ ne représente pas -COOH,
e) au moins un acide monocarboxylique saturé ou insaturé à chaîne linéaire et/ou ramifiée qui est facultativement sulfuré en une quantité qui peut aller jusqu'à 35% en poids ; et/ou un ester de cet acide ; et
f) au moins un triazole de formule : dans laquelle R''₁ représente -COOH ou des dérivés alkylés de celui-ci, ou un alkyle à chaîne courte comportant jusqu'à 5 atomes de carbone ; n représente zéro ou un nombre entier entre 1 et 3, bornes incluses ; et R''₂ représente hydrogène, morpholino, alkyle, amido, amino, hydroxy ou des dérivés alkyl- ou aryl-substitués de ceux-ci ; ou un triazole choisi parmi le 1,2,4-triazole, le 1,2,3-triazole, le 5-anilo-1,2,3,4-thiatriazole, le 3-amino-1,2,4-triazole, le 1-H-benzotriazole-1-yl-méthylisocyanure, le méthylène-bis-benzotriazole et le naphtotriazole ; et
g) au moins un additif extrême-pression contenant du phosphore.
dans laquelle les composants (b) à (g) sont présents dans des quantités choisies de manière à satisfaire à l'exigence de la United States Navy (Marine des Etats-Unis d'Amérique) pour l'essai Ryder effectué à 100°C, de 200 (classement relatif, % Herco® A comme fluide de référence).

2. Composition lubrifiante selon la revendication 1, dans laquelle au moins un matériau de base du composant de base est un ester de polyol.

3. Composition lubrifiante selon la revendication 2, dans laquelle le matériau de base de type ester de polyol comprend un ou plusieurs acides monocarboxyliques en C₅ à C₁₂ estérifiés avec un ou plusieurs polyols ou éthers de polyols.

4. Composition lubrifiante selon l'une quelconque des revendications 1 à 3, dans laquelle le composant de base présente une viscosité située dans la gamme allant de 8,75 à 9,25 mm²/s (cSt) à 100°C.

5. Composition lubrifiante selon l'une quelconque des revendications précédentes dans laquelle l'antioxydant comprend un antioxydant phénolique stériquement encombré présent en une quantité de 0,4 à 0,8% en poids de la composition.

6. Composition lubrifiante selon l'une quelconque des revendications précédentes dans laquelle l'antioxydant comprend un antioxydant de type amine aromatique présent en une quantité de 0,5 à 1,5% en poids de la composition.

7. Composition lubrifiante selon l'une quelconque des revendications précédentes, dans laquelle le composant acide dicarboxylique saturé et/ou insaturé (d) est présent en une quantité allant jusqu'à 0,15% en poids de la composition.

8. Composition lubrifiante selon l'une quelconque des revendications précédentes dans laquelle le composant acide dicarboxylique saturé et/ou insaturé (d) comprend de l'acide sébacique.

9. Composition lubrifiante selon l'une quelconque des revendications précédentes dans laquelle le composant acide monocarboxylique (e) est présent en une quantité de 0,001 à 0,35% en poids de la composition.

10. Composition lubrifiante selon l'une quelconque des revendications précédentes, dans laquelle le composant acide monocarboxylique (e) comprend de l'acide oléique sulfuré.

11. Composition lubrifiante selon l'une quelconque des revendications précédentes, dans laquelle le composant triazole (f) est présent en une quantité de 0,005 à 0,25% en poids de la composition.

12. Composition lubrifiante selon l'une quelconque des revendications précédentes, dans laquelle le composant triazole (f) comprend du benzotriazole.

13. Composition lubrifiante selon l'une quelconque des revendications précédentes, dans laquelle le composant additif extrême-pression (g) comprend un additif extrême-pression phosphate d'amine présent en une quantité de 0,2 à 0,6% en poids de la composition.

14. Composition lubrifiante selon l'une quelconque des revendications précédentes dans laquelle le composant additif extrême-pression (g) comprend un additif extrême-pression phosphorothionate présent en une quantité de 0,5 à 1,5% en poids de la composition.

15. Lubrifiant de transmission pour hélicoptère comprenant les composants (a) à (g) tels que définis dans l'une quelconque des revendications précédentes.
